

## GASOLINE CONTAINING HYDRAZONES

Bruno H. Wojcik, Niagara Falls, N.Y., assignor to Olin Mathieson Chemical Corporation, a corporation of Virginia

No Drawing. Filed Feb. 21, 1956, Ser. No. 566,782

7 Claims. (Cl. 44—63)

This invention relates to improvements in motor fuels, particularly in gasoline fuels for internal combustion engines. More particularly, it relates to improvements effected in gasoline motor fuels by the incorporation therein of minor proportions of hydrazones.

Gasoline suitable for use as a motor fuel is a complex mixture consisting largely of a variety of hydrocarbons and usually includes one or more non-hydrocarbon materials added thereto to improve the storage and operating characteristics of the fuel.

Few modern gasolines are straight run fuels and the mixture usually contains a substantial fraction of hydrocarbons obtained by cracking, isomerization, alkylation, polymerization, reforming, hydroforming or other operations. Many of these processes are designed to produce hydrocarbons which when blended with straight-run gasoline will improve the anti-knock value. While these hydrocarbons have high anti-knock blending value, they are characteristically less stable than the saturated hydrocarbons of straight-run gasoline. The processed hydrocarbons are notably subject to oxidation and polymerization in storage with the formation of gummy products deleterious to storage containers and pumps, as well as feed lines, pump and carburetor in the automotive vehicle. In addition, they may give rise in the engine to materials which at normal temperatures of operation form resinous deposits on pistons, rings, cylinder walls and bearings which interfere with proper operation of the automotive engine. Numerous inhibitors are commercially available for stabilization of gasoline in these respects and to improve storage and operating characteristics of the fuel by avoiding the formation of resinous products of these unstable hydrocarbons. Most of the inhibitors are compounds of relatively high molecular weight compared with gasoline hydrocarbons and are likely to remain as residues on evaporation of the fuel.

Motor gasoline is also usually blended with appropriate portions of a butane fraction, particularly for winter use to provide sufficient volatility for easy starting. Many automotive engines, however, are not maintained in good operating condition and difficult starting is characteristic of such engines even though the refiner provides a suitable fuel for engines in average or better condition. Added tricresyl phosphate is advertised as improving starting characteristics.

Tetraethyl lead is commonly added to improve the anti-knock value of the gasoline and usually a mixture of halogen compounds is simultaneously added to insure the vaporization of the combustion products of the tetraethyl lead. In addition, other materials may be added to gasoline for various purposes including light lubricating oils for upper cylindrical lubrication and many other dopes for various purposes.

The use of unsubstituted hydrazine as an additive is highly impractical as hydrazine is substantially insoluble in hydrocarbons. It cannot, therefore, be incorporated in the fuel, but must be injected at some suitable posi-

tion in the fuel line or air intake by a suitable device. Furthermore, the presence of minor amounts of unsubstituted hydrazine drastically reduces the octane rating of gasoline by 10 or more octane units.

According to the present invention, the addition of minor proportions of hydrazones or mixtures thereof to gasoline surprisingly improves the storage, starting and other operating characteristics of the fuel. The hydrazones fall within the scope of the generic formula:



wherein R<sub>1</sub>, R<sub>2</sub>, R<sub>3</sub> and R<sub>4</sub> are selected from the group consisting of hydrogen, aliphatic hydrocarbon, alicyclic hydrocarbon, aromatic hydrocarbon and heterocyclic substituents. They can be the same or different. In the above formula, the total number of carbon atoms should preferably not exceed 12. Compounds of up to and

including 36 carbon atoms, however, have shown desirable properties and are included in the invention. A wide variety of these hydrazones is known to the art and their method of preparation is old, viz. condensation of an aldehyde or ketone with hydrazine, a suitably monosubstituted hydrazine, or a N,N-disubstituted hydrazine. It is also possible for these substituents to carry various innocuous groups, for example, an hydroxyl group or an ether group. Preferably, R<sub>1</sub>, R<sub>2</sub>, R<sub>3</sub> and R<sub>4</sub> are selected from the group consisting of hydrogen, alkyl, cycloalkyl, aryl and heterocyclics containing one hetero atom.

Examples of some hydrazones encompassed by this invention are:

- 35 1. Acetone hydrazone
2. Formaldehyde dimethylhydrazone
3. Acetaldehyde dimethylhydrazone
4. Formaldehyde diethylhydrazone
5. Acetaldehyde cyclohexylhydrazone
6. Propionaldehyde phenylhydrazone
7. Methyl ethyl ketone dimethylhydrazone
8. Benzaldehyde dimethylhydrazone
9. Benzaldehyde diphenylhydrazone
10. Benzaldehyde cyclopentylhydrazone
11. Benzaldehyde-2-pyridylhydrazone

The hydrazones or mixtures thereof can be dissolved to the extent of 0.1 to 2 percent by weight in gasoline to provide suitable compositions according to the present invention. Somewhat smaller or larger amounts of the hydrazones or mixtures thereof can also be used, but preferably the amount used is within the range of from about 0.5 to 1 percent by weight, based on the gasoline.

55 The presence of hydrazones in gasoline improves its stability towards the action of oxygen in storage. The hydrazones are reactive with dissolved oxygen and prevent its action on the relatively unstable hydrocarbons by reacting more readily with the oxygen dissolved from the air. This activity of the hydrazones may not remove

60 the necessity for incorporation of minor amounts of the usual anti-oxidants but it tends to reduce the quantity required in order to provide satisfactory stability in storage. This in turn reduces the proportion of non-volatile components in the gasoline and effects improvements in the cleanliness of lines, pumps and carburetors in which the gasoline is used.

65 Many hydrazones are sufficiently strong bases to combine with organic acids and they combine with most inorganic acids. Sulfuric acid derived from organic sulfur contained in the fuel or other sources, phosphoric acid or hydrohalogen acids derived from other additives

combine with the hydrazones and are neutralized to form relatively less corrosive salts. This materially reduces corrosion of storage tanks and parts of the automotive vehicle which may be subject to such corrosion. The alkalinity of the hydrazones further effects improvements in reducing engine wear due to the removal or conversion of corrosive acids to relatively less corrosive materials.

Beneficial results are noticeable when as little as 0.1 percent by weight or less of a hydrazone is added and quantities of 2 percent by weight or more can be used if desired. Ordinarily, within this range, material improvements are effected economically by the addition of from about 0.5 to 1 percent by weight of a suitable hydrazone to the gasoline.

The hydrazones can be blended with the gasoline in any convenient manner or at any stage. They can be added as pure compounds or may be diluted with one of the heavier blending stocks to be used.

*Example I*

A solution of 1 percent by weight of acetaldehyde cyclohexylhydrazone in gasoline is an example of this invention.

*Example II*

Another example of this invention is a solution of 1 percent by weight of acetone hydrazone in gasoline.

*Example III*

A blend of .85 percent by weight of benzaldehyde-2-pyridylhydrazone and 99.15 percent by weight of gasoline is a further example of this invention.

*Example IV*

An additional example of this invention is a solution of 2 percent by weight of benzaldehyde dimethylhydrazone and 98 percent by weight of gasoline.

*Example V*

A sample of stock gasoline containing 1 percent by weight of acetaldehyde dimethylhydrazone was tested for its oxygen bomb stability according to ASTM method D525-49. The break point was reached in 960 minutes. Without any acetaldehyde dimethylhydrazone present, this break point was reached in 615 minutes. This indicates that the fuel's resistance to oxidation was considerably increased by the addition of acetaldehyde dimethylhydrazone.

*Example VI*

Two samples of stock gasoline were tested, according to the method of Example V, one with and one without

the addition of 1 percent by weight of benzaldehyde dimethylhydrazone. The break point was reached in 615 minutes without this additive. However, 960 minutes were required to reach the break point with the sample containing the benzaldehyde dimethylhydrazone.

I claim:

1. Gasoline containing as an additive from 0.1 to 2 percent by weight of at least one of the materials falling within the scope of the formula



wherein  $\text{R}_1$ ,  $\text{R}_2$ ,  $\text{R}_3$  and  $\text{R}_4$  are selected indiscriminately from the group consisting of hydrogen, alkyl, cycloalkyl and aryl hydrocarbon radicals and heterocyclic radicals containing one hetero nitrogen atom, with the proviso that the total number of carbon atoms in the material does not exceed 36.

2. The composition of claim 1 in which the gasoline contains about 0.5 to 1 percent by weight of the material.

3. Gasoline containing from 0.1 to 2 weight percent of acetone hydrazone.

4. Gasoline containing from 0.1 to 2 weight percent of acetaldehyde cyclohexylhydrazone.

5. Gasoline containing from 0.1 to 2 weight percent of benzaldehyde-2-pyridylhydrazone.

6. Gasoline containing from 0.1 to 2 weight percent of benzaldehyde dimethylhydrazone.

7. Gasoline containing from 0.1 to 2 weight percent of acetaldehyde dimethylhydrazone.

References Cited in the file of this patent

UNITED STATES PATENTS

|           |          |       |                |
|-----------|----------|-------|----------------|
| 1,906,044 | Burk     | ----- | Apr. 25, 1933  |
| 1,958,744 | Cross    | ----- | May 15, 1934   |
| 2,027,394 | McMullan | ----- | Jan. 14, 1936  |
| 2,055,810 | Bartram  | ----- | Sept. 29, 1936 |
| 2,339,984 | Eitelman | ----- | Jan. 25, 1944  |
| 2,714,057 | Chenicek | ----- | July 26, 1955  |

OTHER REFERENCES

Industrial and Engineering Chemistry, vol. 42, September 1950, "Hydrazine in Organic Chemistry," by Byrkit and Michalek, pp. 1862 to 1875.

"The Chemistry of Hydrazine," by Audrieth and Ogg, Wiley and Sons Inc., 1951, pp. 225, 226 and 227.

Scientific American, vol. 189, No. 1, July 1953, "Hydrazine," by Lessing, pp. 30 to 33.

Journal of Organic Chemistry, vol. 15, 1950, pp. 1125-1130.